# EUROPEAN PATENT SPECIFICATION

(11) **EP 0 873 567 B1**
(45) Date of publication and mention of the grant of the patent: **03.04.2002**
(21) Application number: 97901927.0
(22) Date of filing: 08.01.1997
(51) Int. Cl.: H01F 17/06, H01F 27/25, H01F 27/34, H01F 1/153

(54) **DISTRIBUTED GAP ELECTRICAL CHOKE**
ELEKTRISCHER DROSSEL MIT VERTEILTE SPALT
BOBINE DE REACTANCE AVEC REPARTITION D'ENTREFER

(30) Priority: 11.01.1996 US 584787
(43) Date of publication of application: 28.10.1998
(73) Proprietor: Honeywell International Inc., Morristown, New Jersey 07962 (US)
(72) Inventor: COLLINS, Aliki, Newton, MA 02166 (US); SILGAILIS, John, Cedar Grove, NJ 07009 (US); ABOU-ELIAS, Joseph, Great Meadows, NJ 07838 (US); MARTIS, Ronald, J., East Hanover, NJ 07936 (US); HASEGAWA, Ryusuke, Morristown, NJ 07960 (US)
(74) Representative: Weber, Dieter, Dr.
(86) International application number: US9700178
(87) International publication number: WO9725727

(56) References cited:
- EP-A- 0 513 385
- GB-A- 2 117 979
- US-A- 4 300 950
- IEEE TRANSACTIONS ON MAGNETICS, vol. 20, no. 5, September 1984, NEW YORK US, pages 1415-1416, XP002030239 R.V.MAJOR ET AL : "Development of amorphous Fe-B based alloys for Choke and Inductor Applications"
- JOURNAL OF MAGNETISM AND MAGNETIC MATERIALS, vol. 115, no. 2 / 03, 11 September 1992, pages 245-249, XP000329941 SINGHAL R ET AL: "CRYSTALLIZATION OF GLASSY FE80B20-XSIX(O X 12) ALLOYS"

## Description

### BACKGROUND OF THE INVENTION

### 1. Field Of The Invention:

This invention relates to an amorphous metal magnetic core with a distributed gap for electrical choke applications; and more particularly to a method for annealing the amorphous core to create the distributed gap therein.

### 2. Description Of The Prior Art:

An electrical choke is an energy storage inductor. For a toroidal shaped inductor the stored energy is W=1/2 [(B²A_{c}lₘ)/(2µ₀µᵣ)] where B is the magnetic flux density, A_{c} is the effective magnetic area of the core, lₘ is the mean magnetic path length, µ₀ is the permeability of the free space and µᵣ is the relative permeability in the material.

By introducing a small air gap in the toroid, the magnetic flux in the air gap remains the same as in the ferromagnetic core material. However, since the permeability of the air (µ~1) is significantly lower than in the typical ferromagnetic material (µ ~several thousands) the magnetic field strength(H) in the gap becomes much higher than in the rest of the core (H=B/µ). The energy stored per unit volume in the magnetic field is W=1/2(BH), indicating it is primarily concentrated in the air gap. In other words, the energy storage capacity of the core is enhanced by the introduction of the gap. The gap can be discrete or distributed. A distributed gap can be introduced by using ferromagnetic powder held together with nonmagnetic binder or by partially crystallizing an amorphous alloy. In the second case, ferromagnetic crystalline phases separate and are surrounded by nonmagnetic matrix. This partial crystallization mechanism is utilized in connection with the choke of the present invention.

In US-A-4,812,181 there is disclosed a method for achieving flat magnetization loop by subjecting Fe base amorphous cores to a long term (more than 10 hrs) anneal at temperatures higher than 410 °C. The method disclosed therein includes the step of crystallizing the surface of the amorphous ribbon, thereby applying stress on the amorphous bulk of the ribbon.

In GB 2,117,979A, an electrical choke is made based on heat treating Fe-base amorphous cores. The maximum permeability is reduced to between 1/50 and 1/30 of the original value, (for maximum permeability of 40,000 this treatment results in values ranging from about 800 and 1300) and the amorphous cores exhibit a degree of crystallization, which does not exceed 10% of the volume.

IEEE Transactions on Magnetics, MAG-20 (1984) Sept., No.5, Part 2, NY, USA pages 1415-1416 discusses the development of amorphous Fe-B based alloys for choke and inductor applications. This paper notes a permeability of 200, but at the expense of hight frequency loss characteristics.

European Patent Application EP-A-513-385 discloses iron-base soft magnetic alloys which require Aluminum to inhibit Fe-B crystal formation.

For applications in power supplies for notebook computers and other small devices there is a need for a very small size electrical choke with very low permeability (100-300), very low core losses, high saturation magnetization and which can sustain high DC bias magnetic fields.

### SUMMARY OF THE INVENTION

The invention provides a method for producing an electrical chake as disclosed in claim 1.

The present invention provides electrical chokes having sizes ranging from about 8 mm to 45 mm OD with permeabilities in the range of 100 to 400 and low core losses (less than 70 W/kg at 100 kHz and 0.1T). Advantageously, the magnetic properties are maintained under DC bias (at least 40% of the initial permeability is maintained at a DC bias field of 3980 A/m or 50 Oe).

There is provided by the present invention a method for heat treating Fe base amorphous alloys in a controlled way to partially crystallize the bulk of the amorphous ribbon and generate microgaps in the cores. As a result of the distributed gaps, the aforementioned properties are achieved.

More specifically, there is provided in accordance with the invention a unique correlation between the degree of crystallization and the permeability values. In order to achieve permeability in.the range of 100 to 400, bulk crystallization of the amorphous core is required, preferably of the order of 10 to 25% of the core volume.

In addition, the present invention requires certain annealing temperature and time parameters and degree of control of these parameters in order to achieve the desired choke properties.

### BRIEF DESCRIPTION OF THE DRAWINGS

The invention will be more fully understood and further advantages will become apparent when reference is had to the following detailed description and the accompanying drawings, in which:
Figure 1 is a graph depicting the relation between the permeability of the core and the annealing temperature, the different curves describing material with different crystallization temperatures;
Figure 2 is a graph depicting the relation between the permeability of the cores and the annealing temperature for different annealing times;
Figure 3 is a graph depicting the loading configuration of the cores for the annealing in order to achieve temperature uniformity within a few degrees;
Figure 4 is a graph depicting core loss in W/kg of the cores as a function of the DC bias field and the frequency;
Figure 5 is a graph depicting the permeability of the cores under DC bias field conditions;
Figure 6 depicts a typical cross-sectional Scanning Electron Microscopy (SEM) picture of the ribbon after the annealing; and
Figure 7 describes the permeability as a function of the volume percent of crystallinity.

### DESCRIPTION OF THE PREFERRED EMBODIMENTS

Fig. 1 depicts the permeability of the annealed Fe-base magnetic core as a function of the annealing temperature. The permeability was measured with an induction bridge at 10 kHz frequency , 8-turn jig and 100 mV ac excitation. The annealing time was kept constant at 6 hrs. All the cores were annealed in an inert gas atmosphere. The different curves represent Fe-base alloys with small variations in the chemical composition and consequently small changes in their crystallization temperature. The crystallization temperatures were measured by Differential Scanning Calorimetry (DSC). A reduction in the permeability is observed with increasing annealing temperature for a constant annealing time. For a given annealing temperature the permeabilities scale according to the crystallization temperature, i.e. the permeability is highest for the alloy with the highest crystallization temperature.

Fig. 2 depicts the permeability of the annealed Fe-base cores with the same chemical composition as a function of the annealing temperature. The different curves represent different annealing times. The plot indicates that for temperatures higher than 450 °C the effect of the annealing temperature dominates the effect of the annealing time.

The appropriate annealing temperature and time combination are selected for an Fe-B-Si base amorphous alloy on the basis of the information in Figs. 1 and 2. This selection can be made provided the crystallization temperature (Tₓ) and/ or chemical composition of the alloy is known. For example, for Fe₈₀B₁₁Si₉ which has Tₓ=507 °C in order to achieve permeabilities in the range of 100 to 400 annealing temperatures in the range of 420 to 425 °C for 6 hrs are appropriate.

Referring again to Fig. 1, reproducibility and uniformity for a given permeability value are obtained when a temperature variation of less than one or two degrees is maintained. Special loading configurations have been developed for the annealing process so that the uniformity and reproducibility of the temperature in the oven are established. For a box type inert gas oven wire mesh Al plates(2) are stacked according to Fig. 3 and the arrangement is placed in the center of the oven. The Al plates are the substrates that hold the cores(1) during the anneal.

Typical magnetic characterization data for the chokes, such as core loss and DC bias are shown in Figs. 4 and 5. The core loss data are plotted as a function of the DC bias field and the different curves represent different measuring frequencies. The data shown are for cores with 25 mm OD. An important parameter for the choke performance is the percent of the initial permeability that remains when the core is driven by a DC bias field. Fig. 5 depicts a typical DC bias curve for a core having 35mm OD.

Cross-sectional scanning electron microscopy (SEM) and x-ray diffraction (XRD) were performed to determine the distribution and percent crystallization of the annealed cores. Fig. 6 depicts a typical cross-sectional SEM indicating that both the bulk of the alloy and the surface are crystallized. This is readily distinguished from the method described in US patent 4,812,181, in which only the surface is crystallized.

The volume percent of the crystallization was determined from both the SEM and XRD data and is plotted in Fig. 7 as a function of permeability. For permeabilities in the range of 100 to 400 bulk crystallization in the range of 5 to 30% is required.

Having thus described the invention in rather full detail, it will be understood that such detail need not be strictly adhered to but that further changes and modifications may suggest themselves to one skilled in the art, all falling within the scope of the invention as defined by the subjoined claims.

## Claims

1. A method for producing an electrical choke having a magnetic core consisting of an iron based amorphous metal alloy, the magnetic core having a distributed air gap, comprising the steps of
annealing the choke in a protective atmosphere at temperature and time being selected so that the amorphous metal alloy of the core being partially crystallized above 10% of the volume and having a permeability of from 100 to 400 at 10kHz.

2. The method of claim 1, wherein the amorphous metal alloy is Fe₈₀B₁₁Si₉, said annealing temperature is 425°C and said annealing time is about 6 to 8 hours.

3. The method of claim 1, wherein the amorphous metal alloy is Fe₈₀B₁₂Si₈, said annealing temperature is 455°C and said annealing time is about 4 hours.

4. The method of any of claims 1 to 3, wherein the annealing step in carried out in the absence of a magnetic field.

5. The method of any of claims 1 to 4, wherein said temperature is controlled to within about 2 to 5 degrees Centigrade during said annealing step.

6. The method of claim 5, wherein said annealing step is carried out in a box type convection oven.

7. The method of any of claims 1 to 6, wherein said temperature and time being selected so that about 10 to 25% of the volume of the amorphous metal alloy of the core is crystalline.

8. The method of any of claims 1 to 7, wherein said reaction being selected so that said partial crystallization causes formation of α-Fe and Fe₂B crystal therein.

9. The method of any of claims 1 to 8, comprising the step of coating said core with a thin high temperature resin, which is electrically insulating said core and which maintains core integrity.

10. An electrical choke produced in accordance with the method recited in any of claims 1 to 9.

## Patentansprüche

1. Verfahren zur Herstellung einer elektrischen Drossel mit einem aus einer amorphen Metallegierung auf Eisenbasis bestehenden magnetischen Kern mit einem verteilten Luftspalt, mit den folgenden Schritten:
Glühen der Drossel in einer Schutzatmosphäre bei einer Temperatur und über eine Zeit, die so ausgewählt sind, daß die amorphe Metallegierung des Kerns zu über 10% Vol.-% teilkristallisiert ist und bei 10 kHz eine Permeabilität von 100 bis 400 aufweist.

2. Verfahren nach Anspruch 1, bei dem die amorphe Metallegierung Fe₈₀B₁₁Si₉ ist, die Glühtemperatur 425°C beträgt und die Glühzeit etwa 6 bis 8 Stunden dauert.

3. Verfahren nach Anspruch 1, bei dem die amorphe Metallegierung Fe₈₀B₁₂Si₈ ist, die Glühtemperatur 455°C beträgt und die Glühzeit etwa 4 Stunden dauert.

4. Verfahren nach einem der Ansprüche 1 bis 3, bei dem der Glühschritt in Abwesenheit eines Magnetfelds durchgeführt wird.

5. Verfahren nach einem der Ansprüche 1 bis 4, bei dem die Temperatur während des Glühschritts mit einer Genauigkeit von etwa 2 bis 5 Grad Celsius gesteuert wird.

6. Verfahren nach Anspruch 5, bei dem der Glühschritt in einem kastenartigen Konvektionsofen durchgeführt wird.

7. Verfahren nach einem der Ansprüche 1 bis 6, bei dem die Temperatur und die Zeit so ausgewählt sind, daß etwa 10 bis 25 Vol.-% der amorphen Metallegierung des Kerns kristallin sind.

8. Verfahren nach einem der Ansprüche 1 bis 7, bei dem die Reaktion derart ausgewählt wird, daß die Teilkristallisierung eine α-Fe- und Fe₂B-Kristall-Ausbildung darin bewirkt.

9. Verfahren nach einem der Ansprüche 1 bis 8, mit dem Schritt des Beschichtens des Kerns mit einem dünnen Hochtemperaturharz, das den Kern elektrisch isoliert und die Integrität des Kerns aufrechterhält.

10. Elektrische Drossel, hergestellt nach dem in einem der Ansprüche 1 bis 9 angeführten Verfahren.

## Revendications

1. Méthode pour produire une bobine de réactance électrique ayant un noyau magnétique constitué d'un alliage de métal amorphe à base de fer, le noyau magnétique présentant une répartition d'entrefer, comprenant les étapes de
recuit de la bobine de réactance dans une atmosphère protectrice à une température et pendant une durée déterminées de telle sorte que l'alliage de métal amorphe du noyau soit en partie cristallisé à raison de plus de 10% de son volume et présente une perméabilité allant de 100 à 400 à 10 kHz.

2. Méthode conformément à la revendication 1, dans laquelle l'alliage de métal amorphe est le Fe₈₀B₁₁Si₉, ladite température de recuit est de 425 °C et ladite durée du recuit est d'environ 6 à 8 heures.

3. Méthode conformément à la revendication 1, dans laquelle l'alliage de métal amorphe est le Fe₈₀B₁₂Si₈, ladite température de recuit est de 455°C et ladite durée du recuit est d'environ 4 heures.

4. Méthode conformément à l'une quelconque des revendications 1 à 3, dans laquelle l'étape de recuit est exécutée en l'absence d'un champ magnétique.

5. Méthode conformément à l'une quelconque des revendications 1 à 4, dans laquelle ladite température est contrôlée à l'intérieur d'une gamme d'environ 2 à 5 degrés centigrades durant ladite étape de recuit.

6. Méthode conformément à la revendication 5, dans laquelle ladite étape de recuit est exécutée dans un four à convection de type à cloche.

7. Méthode conformément à l'une quelconque des revendications 1 à 6, dans laquelle ladite température et ladite durée sont sélectionnées de telle sorte qu'environ 10% à 25% du volume de l'alliage de métal amorphe du noyau soient cristallins.

8. Méthode conformément à l'une quelconque des revendications 1 à 7, dans laquelle ladite réaction est sélectionnée de telle sorte que ladite cristallisation partielle provoque la formation de cristal .-Fe et Fe₂B au cours de celle-ci.

9. Méthode conformément à l'une quelconque des revendications 1 à 8, comprenant l'étape de revêtement dudit noyau à l'aide d'une résine fine à température élevée, qui isole électriquement ledit noyau et qui maintient l'intégrité du noyau.

10. Bobine de réactance électrique produite conformément à la méthode décrite dans l'une quelconque des revendications 1 à 9.
